

## UNITED STATES PATENT OFFICE

2,112,756

## MANUFACTURE OF SAFETY PAPER

Viktor T. Bausch, Berlin, and Adolf Schroth, Neu-Kaliss, Mecklenburg, Germany, assignors to Felix Schoeller & Bausch, Mecklenburg, Germany

No Drawing. Application June 23, 1936, Serial No. 86,888. In Germany February 7, 1934

8 Claims. (Cl. 91—67.95)

This invention relates to the manufacture and production of safety papers, for use in preventing the fraudulent alteration of documents.

It is well known to protect documents from falsification by the use of chemicals by means of safety reagents which react with oxidizing agents to produce discolouration. This discolouration can in general be removed more or less easily by reducing agents without leaving any trace.

No safety reagent is yet known which reacts with certainty on the reducing agents which are employed in practice. Mercury sulphonate has, it is true, been previously proposed for this purpose, but, apart from the ease with which it decomposes in air and light, this compound is used less because its reaction with reducing agents is extremely weak. That this must be the case is clear from the fact that organic mercury compounds of this constitution are not true salts in the inorganic sense of the word, but are so-called pseudosalts, in which the mercury is also attached by secondary valencies to other atoms.

As distinguished therefrom, inorganic salts which can be reduced by mild reducing agents, in particular sulphites, to form substances or elements of different colour are employed according to the present invention. These respond instantaneously and with certainty to reducing agents, and, therefore, form reliable and practically useful safety reagents for the detection of reducing agents. Complex salts which contain in the outer sphere a component which is reducible to a substance or element of different colour can also be employed in accordance with the invention. In these true salts the element to be reduced can be present both in the cations as well as in the anions. Further, these salts, in addition to their great reacting power, are also distinguished by their stability and above all by their resistance to decomposition by light. Owing to this stability it is possible to combine these safety reagents with other chemicals, in particular with salts which react on oxidizing agents with the production of discolouration.

Forgers always work with mild reducing agents. These are also the basis of the known commercial erasing liquids. If stronger reducing agents were employed, the paper would also be attacked by them and the forgery would be revealed. Sulphite compounds of all kinds are chiefly employed as the reducing agents. The known safety papers, for example those which contain mercury chloride in addition to salts of nickel and cobalt as well as those which contain bismuth iodide or mercury iodide, do not react at all with such mild reducing agents.

The invention also comprises the use of inorganic salts of the kind set forth which, in addition to the reducible constituent, also contain a constituent which reacts with oxidizing agents to produce a discolouration. By this means the manufacture of papers for documents which are to be safeguarded against falsification is greatly facilitated. The salts in question can be manufactured by suitable choice of the salt-forming constituent; one such salt, for example, is manganese tellurite.

It is, of course, known to add to safety papers reagents which respond to oxidizing agents. As distinguished therefrom, however, the safety paper according to the invention possesses the great advantage that, owing to the addition of a salt which responds both to reducing agents and to oxidizing agents, the protection afforded is increased.

The safety reagents according to the invention can be incorporated with the pulp by precipitation during manufacture or can be precipitated outside the paper pulp and then added to the pulp. They can also be applied by impregnation, spraying, or painting or by printing by any suitable printing process.

*Examples*

1. Mercury-I-tungstate is precipitated in the hollander in known manner from a soluble mercurous salt by means of alkali tungstate and is incorporated in the paper pulp to the extent of about 6%.

2. Freshly precipitated, still moist barium tellurite is worked up with an oily agent in accordance with methods well known in the printing colour art and printed on or applied to the paper.

3. 10% of manganese ferrocyanide is incorporated with the paper pulp by precipitation in the hollander and the finished paper is subsequently impregnated with a concentrated alkaline selenite solution.

4. Manganese tellurite in freshly precipitated condition is incorporated in an amount of about 10% as a suspension with the paper pulp in the hollander.

We claim:

1. In the manufacture of safety paper for the purpose set forth, the step which comprises treating paper material with a reducible inorganic salt resistant to decomposition by light and which upon reduction forms a substance which is of different color than the original salt, said salt being selected from the group consisting of manganese tellurite, barium tellurite, and mercurous tungstate.

ganous tellurite, barium tellurite, mercury-I-tungstate and alkali selenite.

2. In the manufacture of safety paper for the purpose set forth, the step which comprises incorporating with the paper pulp a reducible inorganic salt resistant to decomposition by light and which upon reduction forms a substance which is of different color than the original salt, said salt being selected from the group consisting of manganeseous tellurite, barium tellurite, mercury-I-tungstate and alkali selenite.

3. In the manufacture of safety paper for the purpose set forth, the step which comprises applying to the paper a coating containing a reducible inorganic salt resistant to decomposition by light and which upon reduction forms a substance which is of different color than the original salt, said salt being selected from the group consisting of manganeseous tellurite, barium tellurite, mercury-I-tungstate and alkali selenite.

4. A safety paper containing a reducible inorganic salt resistant to decomposition by light and which upon reduction forms a substance

which is of different color than the original salt, said salt being selected from the group consisting of manganeseous tellurite, barium tellurite, mercury-I-tungstate and alkali selenite.

5. A safety paper for the purpose set forth comprising paper and a safety agent comprising an inorganic salt resistant to decomposition by light and which upon reduction forms a substance which is of different color than the original salt, said salt being selected from the group consisting of manganeseous tellurite, barium tellurite, mercury-I-tungstate and alkali selenite.

6. A method of manufacturing safety paper in accordance with claim 1, wherein the inorganic salt is mercury-I-tungstate.

7. A method of manufacturing safety paper in accordance with claim 1, wherein the inorganic salt is barium tellurite.

8. A method of manufacturing safety paper in accordance with claim 1, wherein the inorganic salt is manganeseous tellurite.

VIKTOR TH. BAUSCH.  
ADOLF SCHRÖTH.